

## UNITED STATES PATENT OFFICE

2,257,871

## INSULATING OIL COMPOSITION

Charles E. Trautman, East McKeesport, Pa., assignor to Gulf Research & Development Company, Pittsburgh, Pa., a corporation of Delaware

No Drawing. Application November 9, 1940,  
Serial No. 365,128

## 4 Claims. (Cl. 252—64)

This invention relates to improved insulating oil compositions and it comprises improved transformer oils and other insulating oil compositions containing in admixture therewith relatively small amounts of trithiophenyl phosphate, the amount of said improvement agent being sufficient to stabilize the petroleum oil against oxidation, particularly against sludge formation, development of acidity and other undesirable changes normally resulting from oxidation of the oil under service conditions and to otherwise improve said oil compositions, said improved insulating oil compositions being highly resistant to such undesirable oxidative changes; all as more fully hereinafter set forth and as claimed.

In the present invention, transformer oils and like insulating oils are improved by incorporating in the oil or oil composition, a small amount of trithiophenyl phosphate, the amount added being sufficient to stabilize the oil against oxidation, as stated ante. And the amounts of such additions necessary to effectively stabilize the usual commercial oils do not exceed 1 per cent by weight of the oil. For instance, by adding 0.1 to 0.5 per cent of trithiophenyl phosphate to transformer oils, I have obtained oil compositions which are stable against oxidation. This is more fully shown post. And as there shown, my new and improved oils are superior to the original oils and have a much higher resistance to sludging and other improved properties.

The improvement agent here used, namely, trithiophenyl phosphate is a well known chemical compound. It is readily soluble in petroleum oils in the amounts here employed and it does not deleteriously affect either the physical or electrical properties of transformer oils when incorporated therein in the amounts necessary for the present purposes.

Further, trithiophenyl phosphate is a substantially neutral compound, having the following structural formula:



This compound is an organic ester of phosphorus which in addition to the phosphorus contains three sulfur atoms all of which are divalent. Thus, it is also a thio-ether compound, each of

the sulfur atoms being joined to a phenyl radical, as shown in the above formula. In fact this compound may be obtained by reacting phenyl mercaptan or its alkali metal salts with phosphorus oxychloride ( $OPCl_3$ ) and recovering the trithiophenyl phosphate so obtained. While this compound is soluble in petroleum oils, it is insoluble in water. And when dissolved in transformer oils in small amounts, it improves their properties as fully shown post. And as there shown, my new and improved compounded oils are superior to the original oils and my compounded oil compositions, because of their superior resistance to oxidation and other improved properties, possess exceptional utility as transformer oils.

In many types of electric transformers the core and windings are immersed in a suitable petroleum oil, which serves as a dielectric and insulating oil and for carrying heat away from the core and windings. The requirements of a transformer oil include good dielectric properties, low viscosity to facilitate heat transfer by convection, low pour point to avoid solidification of the oil by cold, high flash and fire points to minimize danger of fire and explosion and low volatility to reduce vapor losses. In addition, the oil must be resistant to oxidation and sludging, and must be of such character as to resist emulsification with water.

Transformer oils ordinarily are distillate oils refined in such manner as to secure the specified characteristics to as great an extent as possible. Achievement of satisfactory oxidation resistance is difficult, for while oxidative changes are slow, transformer oils are ordinarily expected to remain in service for long periods. Oxidative changes may result in the formation of insoluble matter or sludge. The sludge tends to render the oil more miscible with water, with production of emulsions in the presence of condensed water and a consequent degradation of the dielectric properties of the oil body. The sludge also deposits on the windings and core with reduction of the efficiency of heat transfer. Oxidation of transformer oils tends to be promoted by contact with metals, especially copper and with the usual varnishes and insulating materials.

Various materials have been proposed for incorporation into transformer oils with the object of inhibiting oxidation, and some of these have come into use. The usual anti-oxidants may be divided into two principal classes: (1) those which are associated with a lengthening of the induction period, that is, the time which elapses

before appearance of sludge in the oil subject to oxidation, and (2) those which reduce the rate at which sludge is formed after it once begins to form. In evaluating oils containing anti-oxidants, the most useful criterion is a value which takes into account both of these characteristics viz., the time required, under the test conditions, to form a definite amount of sludge, say, 0.1 per cent by weight of the oil.

I have discovered that trithiophenyl phosphate brings about a lengthening of the induction period and a lessening of the rate of sludge formation thereafter when incorporated in transformer oils even in minimal amounts. As a result of these two inherent properties of trithiophenyl phosphate, compounded transformer oils containing this agent have an improved over-all efficiency under service conditions. And such advantageous improvements can be obtained without deleteriously affecting the electrical and physical properties of the transformer oil. For instance, the resistance of the oil to absorption of moisture and to emulsification are not lowered; trithiophenyl phosphate being insoluble in water as stated ante. If anything, those properties of the transformer oil are also improved by the addition of trithiophenyl phosphate. On the other hand, trithiophenyl phosphate is readily soluble in transformer oils in the amounts necessary to obtain the desired improvements in resistance to oxidation. In other words, trithiophenyl phosphate is fully miscible with such oils initially and compatible with them under service conditions.

That is, I have found that triphenyl phosphate is a useful improvement agent for insulating oils and has several advantages as an improvement agent for such oils, particularly transformer oils.

In preparing my improved transformer oils, various petroleum oils may be employed and the amounts of trithiophenyl phosphate added to the oil may be varied to give the improved stability and other improvements desired. In general, the amounts of trithiophenyl phosphate employed in accordance with my invention are not in excess of 1 per cent by weight on the oil to be inhibited. I have found that 0.1 per cent of trithiophenyl phosphate is effective but this may be varied in accordance with the results desired, although it should not ordinarily be necessary to employ more than 0.5 per cent of trithiophenyl phosphate with the usual transformer oils. Of course, the exact amounts required to secure the desired improvements vary with the particular oil employed.

In the practice of the present invention, the oil bases to which this agent is added are the usual transformer oils ordinarily comprising highly refined petroleum distillates having the physical characteristics within the ordinary specifications for such oils. The acid-refined and solvent-refined oils may be employed. In some instances it is desirable to employ oils which have been subjected both to acid-refining and solvent-refining methods.

By incorporating the said small amounts of trithiophenyl phosphate in such oils, improved insulating oils are readily obtained. The improved oil compositions so obtained are resistant to sludging and other undesirable oxidative changes under service conditions.

The data given in the table post will serve to illustrate the practice of my invention and the utility thereof. The test data given in the table were obtained in accordance with the sludge

formation test for mineral transformer oil, described by F. M. Clark and E. A. Snyder in their paper entitled "Testing for Sludge Formations in Mineral Transformer Oil," presented at the thirteenth annual meeting for the American Society for Testing Materials.

In the tests reported in said table, samples of oil and of the compounded oils were maintained in tubes containing copper wire at a constant 10 temperature of 120° C. The tubes were opened at the top to an enclosed air space and dry air was passed at a controlled rate of 1½ to 2 cubic feet per hour through the enclosed space above the sample tubes. In each tube was introduced 15 22 grams of oil or oil composition to be tested, a number of tubes being employed. At prescribed intervals the tubes were successively removed and the amount of sludge determined. The results of these tests are reported in terms 20 of the induction period, the per cent of sludge formed per day after the induction period and the total number of days required to form 0.1 per cent of sludge.

The oil employed in all of the tests set forth 25 herein below was a typical petroleum transformer oil commonly used for the purpose indicated. The results obtained in testing the oil alone and in testing the oil together with varying amounts of trithiophenyl phosphate are as follows:

30

Table

| 35 | Transformer oil |       | Induction period   | Rate of sludge formation, after induction period | Total time to form 0.1 percent sludge |  |  |
|----|-----------------|-------|--------------------|--------------------------------------------------|---------------------------------------|--|--|
|    | Composition     |       |                    |                                                  |                                       |  |  |
|    | No.             | Oil   | T. T. P. phosphate |                                                  |                                       |  |  |
| 40 | 1               | Parts | Parts              | Days                                             | Per cent per day                      |  |  |
|    | 1               | 100   | 0.5                | 0.5                                              | 0.0100                                |  |  |
|    | 2               | 99.9  | 0.1                | 1.5                                              | 0.0085                                |  |  |
|    | 3               | 99.7  | 0.3                | 3.0                                              | 0.0065                                |  |  |
|    | 4               | 99.5  | 0.5                | 6.0                                              | 0.0060                                |  |  |
|    |                 |       |                    |                                                  | Days                                  |  |  |

In the above table, the "Parts" are parts by weight and the abbreviation "T. T. P. phosphate" represents trithiophenyl phosphate.

From the data given in the above table, it is evident that my improved transformer oils containing trithiophenyl phosphate are superior to the original transformer oil. For instance, by 50 comparing the results obtained with the original oil No. 1 against those obtained with the transformer oils 2, 3 and 4 (made in accordance with the present invention) it will be seen that my improved transformer oils are much more stable 55 against sludging than the original oil.

For one thing, my improved oils have an induction period greater than that of the original oil. For example, my improved transformer oil No. 2 has an induction period three times that of the original oil. That is, even as little as 0.1 per cent of trithiophenyl phosphate inhibits oxidation. And by adding larger amounts, further improvements can be obtained. This is shown in the case of oils Nos. 3 and 4 which contain 0.3 to 0.5 per cent, respectively, and show induction period six and twelve times greater than that of the original oil.

Another and even more important improvement obtainable by means of trithiophenyl phosphate is shown by the data on the rate of sludge formation given in the table. As shown by that data, the incorporation of small amounts of trithiophenyl phosphate in the oil markedly decreases the rate of sludge formation after the induction period. For example, by comparing oil

No. 2 with the original oil (No. 1), it will be seen that as little as 0.1 per cent of trithiophenyl phosphate decreases the rate of sludge formation approximately 15 per cent. By increasing the amount of trithiophenyl phosphate added, the rate of sludge formation may be further decreased. For instance, in the case of oils Nos. 3 and 4, which contain 0.3 and 0.5 per cent of trithiophenyl phosphate, by weight on the oil, there is a 35 and 40 per cent reduction in the rate of sludge formation, respectively. In other words, my improved transformer oils containing small amounts of trithiophenyl phosphate dissolved therein form much less sludge per day than the original oil.

Thus my improved transformer oils have a longer induction period and a much lower rate of sludge formation after the induction period than the original oil. Consequently they have a much greater resistance to sludging, and this over-all superiority is evident from the data on the total time to form 0.1 per cent sludge given in the table. For example, transformer oils 2, 3 and 4 are from 40 per cent to 180 per cent more resistant to sludging than the original oil, as determined by said accelerated test and expressed in terms of the total time to form 0.1 per cent sludge.

From the facts and data given ante, it is evident that my improved transformer oils containing trithiophenyl phosphate are much superior to the original transformer oil as to resistance to sludging and other oxidation changes.

While my invention has been described herein and illustrated ante with particular reference to transformer oil compositions, trithiophenyl phosphate is equally effective in stabilizing other electrical insulating oils against oxidation and deterioration. And in addition to improving trans-

former oils, I can also improve other insulating oils by the present invention.

In improving insulating oils generally, I likewise incorporate small amounts of trithiophenyl phosphate in the oil. The amount added to the oil may be varied according to the particular insulating oil employed to obtain the improvement desired. By the present invention, various types of insulating oils, such as cable oils, switch oils, circuit breaker oils, etc., as well as transformer oils, may be improved by incorporating sufficient trithiophenyl phosphate in the oil to render it highly resistant to sludging and other deleterious oxidation changes under service conditions, without deleteriously affecting the electrical and physical properties of the oil necessary for the various uses thereof as an insulating oil.

What I claim is:

1. In the operation of electrical transformers containing a petroleum oil as a dielectric and cooling medium, the improvement which comprises maintaining a small amount of trithiophenyl phosphate in said oil to substantially inhibit oxidation changes which would otherwise take place in said oil during normal conditions of such use.
2. The process of claim 1 wherein the amount of trithiophenyl phosphate maintained in said oil is from 0.1 to 0.5 per cent of the oil.
3. In the operation of electrical transformers containing a petroleum oil as a dielectric and cooling medium, the improvement which comprises insulating and cooling the windings and core of the transformer with a petroleum oil containing a small amount of trithiophenyl phosphate dissolved therein.
4. The process of claim 3 wherein said petroleum oil contains 0.1 to 0.5 per cent of trithiophenyl phosphate.

CHARLES E. TRAUTMAN.